

Dec. 17, 1963

**E. J. GRISET, JR.**

**3,114,235**

## METHOD OF FORMING A ROUND COLLAGEN STRAND

Original Filed April 13, 1959

4 Sheets-Sheet 1



INVENTOR.  
ERNEST J. GRISSET JR.

BY Robert W. Kell

**ATTORNEY**

Dec. 17, 1963

E. J. GRISSET, JR

3,114,235

METHOD OF FORMING A ROUND COLLAGEN STRAND

Original Filed April 13, 1959

4 Sheets-Sheet 2



INVENTOR.  
ERNEST J. GRISSET JR  
BY Robert W. Kell

ATTORNEY

Dec. 17, 1963

E. J. GRISET, JR

3,114,235

METHOD OF FORMING A ROUND COLLAGEN STRAND

Original Filed April 13, 1959

4 Sheets-Sheet 3

*Fig. 5.*



INVENTOR.  
ERNEST J. GRISET, JR.  
BY *Robert W. Bell*  
ATTORNEY

Dec. 17, 1963

E. J. GRISSET, JR

3,114,235

METHOD OF FORMING A ROUND COLLAGEN STRAND

Original Filed April 13, 1959

4 Sheets-Sheet 4



Fig. 6.

INVENTOR.  
ERNEST J. GRISSET, JR.  
BY *Robert W. Kell*

ATTORNEY

**1**

3,114,235

**METHOD OF FORMING A ROUND COLLAGEN STRAND**

Ernest J. Griset, Jr., Bound Brook, N.J., assignor to

Ethicon, Inc., a corporation of New Jersey

Original application Apr. 13, 1959, Ser. No. 806,067.  
Divided and this application Dec. 1, 1960, Ser. No. 72,987

4 Claims. (Cl. 57—157)

This invention relates to a method of treating collagen multifilament and more particularly to methods for improving the roundness and physical properties of extruded collagen sutures.

For the sake of clarity, the terms used herein are defined as follows:

The term "native collagen fiber," as used herein, means a thread-like collagen structure as it exists in connective tissue.

The term "swollen collagen fibrils," as used herein, means a thread-like collagen structure that has been swollen in acid solution to a diameter of about 200 to 2000 Angstrom units.

The term "monofilament," as used herein, means a single thread of oriented collagen fibrils as extruded through a single orifice in a spinnerette.

The term "multifilament," as used herein, means a group of individual separate filaments or incompletely bonded filaments that have been extruded through a spinnerette.

The term "open multifilament" as used herein means a fluffy multifilament, the bulk of which is large due to the separation of adjacent monofilaments.

The term "ribbon," as used herein, means a thin film of oriented collagen fibrils, for example, as extruded through a slit.

The term "multiribbon," as used herein, means a group of individual ribbons extruded through a plurality of slits.

The term "strand," as used herein, means a group of filaments or ribbons that have been united to form a bonded structure.

The term "cord," as used herein, means a group of filaments or ribbons that have been twisted together and are bonded or partially bonded.

Practically the entire production of absorbable sutures and ligatures is currently made from sheep or beef gut by a process that is time consuming and expensive, and yet is not adapted to produce a uniform product. The percent of production that is rejected, therefore, for some defect such as lack of tensile strength or lack of uniformity, is large. The starting material, e.g., sheep intestines, is available only in limited quantities and one can not predetermine the exact size of the finished product.

In view of the obvious deficiencies of such surgical catgut and the disadvantages of the present method of manufacture, many attempts have been made to obtain a better product by treating collagen to form a swollen fibrous mass that is extruded into a dehydrating bath. It has been found necessary to stretch the extruded collagen to orient it as unoriented collagen lacks the strength that is required of a suture. Extruded collagen is quite fragile as it leaves the dehydrating bath and often breaks upon stretching. In addition, the tension causes the extruded collagen to flatten and become deformed through contact with the godets of the spinning machine unless steps are taken to prevent this.

It is an object of the present invention, therefore, to stretch an extruded collagen multifilament or multiribbon without breaking it.

It is also an object of this invention to prepare a round

**2**

collagen strand or cord that is of uniform cross-section throughout its length.

It is another object of the present invention to control the amount of moisture in an extruded collagen multifilament, multiribbon, strand or cord.

Still another object of the present invention is to produce a cord of collagen multifilament or multiribbon.

I have now discovered a method of subjecting a continuously moving wet collagen multifilament, ribbon, multiribbon or strand to a wringing action, whereby the amount of moisture in the collagen is controlled. I do this by the use of a device called a false twister that automatically imparts a false twist to the strand. A false twist may be defined as a twist whose direction on one side of a point of contact is reversed on the opposite side, thus cancelling the twist. By varying the speed of the false twister, I can adjust the moisture in the collagen multifilament, ribbon, multiribbon or strand and thereby the tension during the spinning process. The amount of moisture that is present in the extruded collagen is quite important, as moisture decreases the tensile strength so that a wet collagen product can not be stretched sufficiently without breaking.

In addition, twisting a collagen multifilament, ribbon, multiribbon or strand as it leaves the dehydrating bath increases the strength of the moving collagen at the place where it is weakest.

The method of operating the false twister may be varied in accordance with the present invention to achieve different results. Thus, the speed of the false twister is one of the spinning conditions that determines the extent to which the multifilament is united to form a strand. If the false twister rotates slowly in a humid atmosphere, a strand is obtained, but the drier the atmosphere, the less the tendency to bond. If it rotates rapidly in a moist atmosphere, the tendency not to bond, which results from the rapid rotation, is compensated for by the moisture and bonding is achieved.

The invention will appear more clearly from the following detailed description when taken in connection with the accompanying drawings, which show, by way of example, a preferred embodiment of the inventive idea.

Referring now to the drawings,

FIGURE 1 is a schematic view of the one form of spinning machine that may be used in the manufacture of continuous collagen multifilaments or strands.

FIGURE 2 is a perspective view of a false twister which is used to wring moisture out of the multifilament and to round the strand during the spinning process.

FIGURE 3 is another perspective view of the false twister of FIGURE 2.

FIGURE 4 is a sectional view of the false twister illustrated in FIGURE 3.

FIGURE 5 is a perspective view of an improved false twister.

FIGURE 6 is a sectional view of the false twister illustrated in FIGURE 5 showing a gear driving means.

Throughout the present specification, collagen multifilament that is traveling from the spinnerette, through the spinning column, over the idler pulley 137, around guide 138, and prior to contact with godet 101, will be referred to as "in the extrusion stage."

Collagen multifilament, or strand, that is traveling between godet 101 and idler pulley 139, and prior to contact with godet 102, will be referred to as "in the first stretching stage."

Collagen multifilament, strand or cord that is traveling between godet 102, around the idler pulleys 135 and 136, and prior to contact with godet 103, will be referred to as "in the second stretching stage."

Referring now to FIGURE 1 of the drawings, which illustrates a vertically upward spinning machine, there are

three godets 101, 102 and 103, of equal circumference (about 3 inches), and they may be made of nylon. It will be noted that the collagen dispersion in a reservoir 114 is maintained under a pressure that is continuously indicated by a gauge 141. This dispersion is forced by a pump 115 through homogenizing jets 116 and 117 and a filter and is extruded vertically upward through a recirculating dehydrating bath 145, over an idler pulley 137, around a guide 138 and onto godet 101. The extruded collagen is pulled vertically upward out of the bath by godet 101.

The extruded collagen 146, as it leaves the dehydrating bath 145 and passes through the extrusion stage, is quite moist, so that there is very little tension between the idler pulley 137 and the guide 138.

The collagen multifilament is wrapped three times around godet 101 before passing to the first stretching stage. Three wraps are sufficient to prevent slippage because the collagen is wet as it reaches this point. At the end of the first stretching stage, however, the collagen is comparatively dry, so that about twelve wraps around the godet 102 are required to prevent slippage.

In the first stretching stage, a false twister 112 twists the collagen multifilament as it leaves godet 101, and thus improves the tensile strength throughout the portion of the multifilament extending from the top of the false twister 112 to the godet 101. It is this section of the extruded collagen that is most weak because of occluded moisture, and the twist imparted by the false twister 112 prevents breaks that would otherwise occur as the collagen multifilament leaves the godet 101. The false twister 112 also wrings the moisture out of the multifilament and, together with a heater 133, controls the moisture content of the collagen multifilament.

In the first stretching stage, the collagen multifilament may be partially rounded and partially bonded by the false twister to form a strand. The amount of bonding that occurs in the first stretching stage may be increased by wetting out the multifilament at godet 101 with water and operating in a moist atmosphere (between 30 and 60 grains of moisture per pound of dry air). It is customary, however, to spin in a dry atmosphere (less than 20 grains of moisture per pound of dry air), and, under these conditions, there is little or no bonding of the collagen multifilament in the first stretching stage.

As pointed out above, the speed of the false twister 112 controls the amount of moisture in the collagen multifilament, and thereby effects the tension as registered by a tensiometer 142 and the amount of stretch that may be applied without breaking the strand. The speed at which the false twister is operated depends upon the relative humidity of the spinning atmosphere, the size (cross-sectional area) of the collagen multifilament or strand, and the character of the collagen dispersion.

I have noted that increasing the speed of the false twister tends to reduce the amount of bonding and a dry open multifilament is collected on godet 102 if the moisture content of the atmosphere is kept low.

On the other hand, operating the false twister at a slower speed will result in partial or complete bonding if the multifilament or atmosphere is moist.

The stretch imparted between godets 101 and 102 provides orientation of the drying multifilament or strand and improves the tensile strength.

When the false twisters 112 and 113 are operated properly, spinning conditions may be controlled so that godet 101 is operated at 10 r.p.m., godet 102 is operated at 14 r.p.m., and godet 103 at 15 r.p.m. Under these conditions, one would obtain, in addition to the 40% stretch between godets 101 and 102, another 10% stretch between godets 102 and 103. The over-all stretch is preferably varied from about 20% to 50%. Since the optimum amount of stretch will result in maximum strength, the machine is preferably operated to give a

stretch somewhat less than that required to break the filaments of the strand.

In the second stretching stage, the moving multifilament or strand is continuously washed and/or tanned by contact with a downward flow of tanning solution 144 in a direction opposite to the direction of strand travel. The wetted out strand from a freely rotating idler pulley 132 is returned to an idler pulley 105 and contacts the tanning bath a second time. In its wet condition, the tanned strand is stretched an additional 10% by the more rapidly rotating godet 103.

The problem in the second stretching stage is to completely bond the multifilament to form a strand that is round. Multiple passages over the circular godet surfaces, especially when the filaments are under tension, forms a flattened strand. The deformation takes place most readily when the strand is wettest, as it leaves the spin bath and tanning bath. Moisture, however, is required to bond together the collagen filaments to form a unitary strand.

In the practice of the present invention, this problem has been solved by using a false twister 113 to place a twist in the strand. The twist backs up to the idler pulley 135 and as the wet strand emerges from it, a gradual tapering takes place which rounds the strand and wrings out the moisture. By locating the idler pulley 135 a sufficient distance above the false twister 113 (preferably about 4 feet) so that the strand is quite dry when it contacts the false twister, I have found that the roundness may be permanently bonded into the strand and is not removed as the resulting cord passes below the false twister. If necessary, a heater 134 may be directed to dry the strand below the false twister and permanently set the uniform circular cross-section that is characteristic of the strand above the false twister 113. The wringing action during the formation of the twist assists in drying the strand.

A preferred type of false twister characterized by three idler pulleys rotating in a common plane, is illustrated in FIGURES 5 and 6 of the drawings.

In these figures, 1 represents the twister head, 2 the hollow vertical drive shaft, 3 the horizontal drive shaft, 4 ball bearings for the shaft 3, 5 ball bearings for the shaft 2, 6 the bevel gear fixed to the horizontal shaft 3, 45 7 the hollow bevel gear fixed to the shaft 2, 8 and 9 the small rollers, 13 the axis of roller 10, 11 and 12 the axes of rollers 8 and 9, 10 the large roller, 14 the multifilament, ribbon, multiribbon or strand, and 15 is one of several set screws that fix the twister head 1 to the hollow vertical drive shaft 2.

The arrows in FIGURE 5 indicate the relative motion of the multifilament and the twister head. It has been found advantageous to allow the multifilament to traverse the false twist mechanism in the direction indicated, since in such use, it passes in a highly twisted condition through the hollow bore of the vertical shaft 2.

The central guidance of the multifilament is obtained by placing the rollers 8 and 9 on their axes 11 and 12 at right angles with the axis of rotation of the vertical shaft 2 in such a manner that the perimeter of each roller is approximately tangential to the axis of rotation of the vertical shaft.

The large roller 10 is disposed between the rollers 8 and 9 on the axis 13, which is parallel with the axes 11 and 12 but offset therefrom. Thus the rollers 8, 9 and 10 rotate in a common plane, but the position and diameter of the roller 10 is so chosen that the path of travel of the multifilament 14 deviates at roll 10 from straight line travel along the axis of rotation of shaft 2 by a distance of the order of  $\frac{1}{2}$  inch. The dimensions of the rollers 8, 9 and 10 and the eccentricity of the axis 13 are not critical as it is only necessary to provide sufficient frictional engagement of the multifilament 14 to twist the same when the twister head 1 is rotated. FIGURES 2 through 4 illustrate an alternate type of false twister that may be

used in the practice of the present invention. The false twister of FIGURE 2 is air driven by a jet of air from the nozzle 16, which is intercepted by the vanes 17, thereby causing rotation of the gear 18. This gear 18 meshes with the upper flange 19 of the false twister 20 and causes rotation thereof in the direction shown.

As indicated in FIGURE 3, the false twister may be constructed with a slot 21 extending from the central opening and vertical axis of the twister 22 to the circumference of the twister head 23. This slot facilitates threading the false twister in the event that the collagen strand breaks during processing.

The preferred shape of the roller 24 is best shown in FIGURE 4. The conical taper from the inner flange 25 of the roller 24 to the outer flange 26 minimizes abrasion of the collagen strand as it passes through the false twister.

The operation of the false twisting device per se and in conjunction with the procedures applied to collagen multifilaments is believed to be apparent from the foregoing description and no further elucidation is deemed necessary as those skilled in the art will now understand how the false twister operates. It will also be understood by those skilled in the art that the false twister will operate to round and dry not only collagen multifilament but also collagen ribbon and collagen multiribbon.

The false twister illustrated in FIGURE 5 is particularly well adapted to the manufacture of round collagen strands from collagen multifilament according to the spinning scheme illustrated in FIGURE 1. For this particular use, when the rate of spinning is about 30-50 inches per minute, the false twisters may be rotated about 100 r.p.m. to 1000 r.p.m. When spinning a size 5/0 strand, both false twisters may be operated at about 600-900 r.p.m. During the manufacture of a larger strand (size 2/0), the speed of both false twisters is preferably reduced to about 400 r.p.m. As mentioned above, the speed of the false twisters may be varied to compensate for spinning conditions. If bonding is obtained, when an open multifilament is desired, the speed of the false twisters may be increased. Slower rotation of the false twisters provides the best conditions for bonding and rounding the strand.

The tensiometers 142 and 143 shown in FIGURE 1 measure tension placed on the dry multifilament strand by godets 102 and 103. The tension effected by godet 102 varies from 10 to 300 grams with the humidity, temperature, speed of the false twister and other operating conditions. These operating variables are preferably adjusted to spin with a tension of between 75 and 150 grams. The tension on the dry strand effected by godet 103 is between 200 and 500 grams. The dried strand is removed from godet 103 by the takeup spool at approximately 45 inches per minute.

It has been observed that atmospheric humidity, a variable during the spinning of a strand, plays an important part in the stretch, the final tensile strength and the bonding of the collagen multifilament to form a strand. If the atmospheric humidity is sufficiently low, an open multifilament may be collected. The humidity is preferably controlled by encasing the spinning operation within the smallest practical enclosure. Air of controlled humidity is introduced into this enclosure to replace the humidity of the building atmosphere with the humidity of a compressed air system. Superior bonded strands are spun when the humidity is controlled between 30 and 60 grains of moisture per pound of dry air. Multifilaments may be spun when the humidity is less than 20 grains per pound. When the humidity is above 60 grains of moisture per pound, the filaments are soft and it is difficult to maintain spinning tension.

The spinning of the dispersion of swollen collagen fibrils to produce a round bonded strand having outstanding properties will be illustrated by Example I. In Example II, the false twister is operated in a dry atmosphere to produce an open unbonded collagen multifilament.

In the examples, all quantities are expressed in parts by weight unless otherwise indicated.

#### Example I

5 A collagen dispersion, prepared as described in U.S. Patent No. 2,919,998 is deaerated under vacuum for 4 hours, aged for 31 hours at 25° C. and 16 hours at 5° C., and then spun in the vertically upward spinning machine illustrated in FIGURE 1. The pressure in the dispersion reservoir as indicated by the pressure gauge 141 is 15 pounds. The pump 115 is operated to extrude 2.82 milliliters of the dispersion each minute. The pressure at the filter, as measured by the gauge 119 is approximately 10 pounds. The spinnerette employed may be a 10 brass plate drilled with 40 openings arranged in three concentric circles. The acetone dehydrating bath is continuously circulated to the spinning column at the rate of about 900 milliliters per minute.

The speed of the godets 101, 102 and 103 is maintained at 10, 13.5 and 14 r.p.m., respectively. The false twisters 112 and 113 are both rotated at 600 r.p.m. The strand is continuously tanned at godet 102 by contacting an aqueous solution containing 4 milliliters of 40% aqueous formaldehyde and 1 gram of aluminum ammonium sulfate per liter, which solution is circulated at the rate of 50 cubic centimeters per minute (25 cubic centimeter per minute through each jet). The blower 113 is adjusted to maintain a tension of 45 to 50 grams as indicated by the tensiometer 142. The blower 134 is directed above the false twister 113 in a manner such that the tension indicated by the tensiometer 143 is about 190 grams. The humidity is maintained at about 30 grains of moisture per pound of dry air throughout the spinning.

35 Under these conditions, the wet tanned strand dries out before the reverse twist is applied by false twister 113. Since the strand is substantially dry at the point of contact with the false twister, the roundness imparted to the strand when wet is not removed.

40 The spinning machine operates continuously and without any difficulties, such as broken strands, under these conditions. The rate of takeup at the spool 147 is about 42 inches per minute. At the end of 6 hours continuous spinning, about 1300 linear feet of a round and 45 uniform collagen bonded strand (size 5/0, 244 denier) is collected.

45 The tensile strength characteristics of this product exceed the requirements set out in the Pharmacopeia of the United States, Vol. XV, page 708.

#### Example II

50 A collagen dispersion (0.86% solids) is spun in the vertically upward spinning machine illustrated in FIGURE 1. The pump 115 is operated to extrude 19.1 milliliters of the dispersion each minute. The spinning column used has an inside diameter of 1 1/16 inches, and the acetone dehydrating bath is circulated through this spinning column at the rate of about 2380 milliliters per minute. The multifilament that emerges from the dehydrating bath is wrapped 1 1/2 times around the godet 101 and passes to the false twister 112. To avoid bonding of the multifilament, a dry atmosphere is maintained (less than 20 grains of moisture per pound of dry air), and the false twister 112 is rotated at 200 r.p.m. The speed of godets 55 101 and 102 is maintained at 10 and 13 r.p.m., respectively, thus producing a stretch between godets 101 and 102 of 30%. Heat is applied by the heater 133 below false twister 112, and the dried multifilament is wrapped 12 times around the godet 102. From godet 102, the multifilament passes directly to the takeup spool. This multifilament may be wet out, tanned, stretched, and bonded as described in Example I above to form a strand (size 2/0), that is equivalent in all respects to cat gut manufactured from intestines.

75 While the description above refers specifically to the

extrusion and treatment of multifilament, it will be recognized that a ribbon or multiribbon may be extruded in a similar manner and process with only minor modifications in the machine illustrated in FIGURE 1, such as using a spinnerette with one or more slots instead of the orifices.

The addition of a bonding agent to the collagen filaments or ribbons is not required because the individual collagen filaments will adhere to each other in the wet stage. Bonding agents may, however, be used in the practice of the present invention when it is desired to manufacture with the false twisters a round strand of fibrils, filaments or ribbons that would not adhere to each other in the absence of a bonding agent, or because of the employment of operating conditions which would otherwise produce only an incompletely bonded multifilament.

The necessity of completing the bonding step before the reverse twist is applied will, of course, be appreciated.

While the invention has been described in detail according to the preferred manner of carrying out the process and yielding the products, it will be obvious to those skilled in the art, after understanding the invention, that changes and modifications may be made therein without departing from the spirit or scope of the invention, and it is intended in the appended claims to cover such changes and modifications.

The present application is a division of application Serial No. 806,067, filed April 13, 1959, now abandoned.

What is claimed is:

1. In the method of manufacturing a round collagen strand of uniform cross-section throughout its length, the steps which include twisting a multiplicity of wet collagen monofilaments to wring out excess moisture and to bond the monofilaments into a unitary structure, drying the monofilaments while in the twisted condition, and removing the twist.

2. A method of bonding and rounding wet collagen ribbon to form a suture which comprises the steps of twisting the wet collagen ribbon to wring out excess moisture, drying the collagen ribbon while in the twisted condition to form a bonded unitary structure of circular cross-section and removing the twist.

3. A method of bonding and rounding a wet collagen multifilament to form a strand which comprises the steps of:

- 10 (a) twisting the collagen multifilament in its wet state to wring out excess moisture;
- (b) drying the collagen multifilament while in the twisted condition to form a strand of circular cross-section, the filaments of which are firmly bonded together; and,
- (c) untwisting the dried collagen strand.

4. A method of manufacturing a collagen strand which comprises the steps of:

- 20 (a) twisting wet collagen multifilament to wring out excess moisture;
- (b) drying the filaments while in the twisted condition; and,
- (c) removing the twist.

25 **References Cited in the file of this patent**

**UNITED STATES PATENTS**

|           |               |       |               |
|-----------|---------------|-------|---------------|
| 2,357,503 | Cidonio       | ----- | Sept. 5, 1944 |
| 2,485,957 | Cresswell     | ----- | Oct. 25, 1949 |
| 2,946,181 | Tissot et al. | ----- | July 26, 1960 |

|         |         |       |                |
|---------|---------|-------|----------------|
| 154,341 | Austria | ----- | Sept. 26, 1938 |
| 558,917 | Belgium | ----- | July 31, 1957  |

(Corresponding to Great Britain No. 814,637, June 10, 1959)

**FOREIGN PATENTS**